

# United States Patent [19]

Mitchell

[11] Patent Number: 4,734,352

[45] Date of Patent: Mar. 29, 1988

[54] POLYHYDROXY CHARGING ADJUVANTS  
FOR LIQUID ELECTROSTATIC  
DEVELOPERS

[75] Inventor: Robert D. Mitchell, Wilmington,  
Del.

[73] Assignee: E. I. Du Pont de Nemours and  
Company, Wilmington, Del.

[21] Appl. No.: 854,610

[22] Filed: Apr. 22, 1986

[51] Int. Cl.<sup>4</sup> ..... G03G 9/12

[52] U.S. Cl. ..... 430/115; 106/20;  
106/23; 106/32

[58] Field of Search ..... 430/115; 106/20, 23,  
106/32

[56] References Cited

U.S. PATENT DOCUMENTS

3,144,184 3/1979 Takahata et al. .  
3,507,679 4/1970 Metcalfe et al. ..... 430/115 X  
3,578,593 5/1971 Hulse .  
3,692,520 9/1972 Mammino et al. .  
3,701,731 10/1972 Hercock et al. .  
3,856,692 12/1974 Mammino et al. .

4,024,292 5/1977 Lu et al. ..... 430/115 X  
4,457,995 7/1984 Ikenoue et al. ..... 430/115

## OTHER PUBLICATIONS

Findlay et al, "Ink for Electrophotographic Imaging",  
IBM Tech. Discl. Bull., vol. 17, No. 7, Dec. 1974, p.  
2117.

Primary Examiner—Roland E. Martin

[57] ABSTRACT

Electrostatic liquid developer having improved charging  
characteristics consisting essentially of

- (A) nonpolar liquid having a Kauri-butanol value of less  
than 30, present in a major amount,
- (B) thermoplastic resin particles having an average by  
area particle size of less than 10  $\mu$ m.
- (C) nonpolar liquid soluble ionic or zwitterionic com-  
pound, and
- (D) a polyhydroxy compound, preferably soluble in the  
developer in an amount of at least 2% by weight.

The electrostatic liquid developers are useful in copying  
making proofs including digital color proofs, litho-  
graphic printing plates, and resists.

15 Claims, No Drawings

**POLYHYDROXY CHARGING ADJUVANTS FOR  
LIQUID ELECTROSTATIC DEVELOPERS**

**DESCRIPTION**

**1. Technical Field**

This invention relates to an electrostatic liquid developer having improved charging characteristics. More particularly this invention relates to an electrostatic liquid developer containing as a constituent a polyhydroxy compound.

**2. Background Art**

It is known that a latent electrostatic image can be developed with toner particles dispersed in an insulating nonpolar liquid. Such dispersed materials are known as liquid toners or liquid developers. A latent electrostatic image may be produced by providing a photoconductive layer with a uniform electrostatic charge and subsequently discharging the electrostatic charge by exposing it to a modulated beam of radiant energy. Other methods are known for forming latent electrostatic images. For example, one method is providing a carrier with a dielectric surface and transferring a preformed electrostatic charge to the surface. Useful liquid toners comprise a thermoplastic resin and dispersant nonpolar liquid. Generally a suitable colorant is present such as a dye or pigment. The colored toner particles are dispersed in the nonpolar liquid which generally has a high-volume resistivity in excess of  $10^9$  ohm centimeters, a low dielectric constant below 3.0 and a high vapor pressure. The toner particles are less than  $10 \mu\text{m}$  average by area size. After the latent electrostatic image has been formed, the image is developed by the colored toner particles dispersed in said dispersant nonpolar liquid and the image may subsequently be transferred to a carrier sheet.

Since the formation of proper images depends on the differences of the charge between the liquid developer and the latent electrostatic image to be developed, it has been found desirable to add a charge director compound to the liquid toner comprising the thermoplastic resin, dispersant nonpolar liquid and generally a colorant. Such liquid toners, while developing good quality images, still do not provide the quality images required for certain end uses, e.g., optimum machine performance in digital color proofing. As a result much research effort has been expended in providing new type charge directors and/or charging adjuvants for electrostatic liquid toners. Higher quality image development of latent electrostatic images is still desired.

It has been found that the above disadvantages can be overcome and improved electrostatic liquid toners prepared containing an ionic or zwitterionic compound soluble in nonpolar liquid which give higher particle mediated conductivity and/or improved image quality on latent electrostatic images.

**3. Disclosure of the Invention**

In accordance with this invention there is provided an electrostatic liquid developer having improved charging characteristics consisting essentially of

- (A) nonpolar liquid having a Kauri-butanol value of less than 30, present in a major amount,
- (B) thermoplastic resin particles having an average by area particle size of less than  $10 \mu\text{m}$ ,
- (C) nonpolar liquid soluble ionic or zwitterionic compound, and
- (D) a polyhydroxy compound.

Throughout the specification the below-listed terms have the following meanings:

Particle mediated conductivity is the difference between the bulk conductivity of the toner and the conductivity of the solution, e.g., carrier or nonpolar liquid.

Bulk conductivity is the conductivity of the developer and may be expressed as BULK.

Conductivity of the solution means the conductivity of the supernatant remaining after centrifugation and may be expressed as SOLN.

Conductivity attributed to the particles is the difference between the bulk conductivity and the conductivity of the solution (BULK-SOLN) and may be expressed as PART.

The electrostatic liquid developer, as defined above consists essentially of the four components more specifically described below. The term "consisting essentially of" means the composition of the electrostatic liquid developer does not exclude unspecified materials which do not prevent the advantages of the developer from being realized. Additional components, in addition to the four primary components, include but are not limited to: colorants such as pigments or dyes, fine particle size oxides, metals, etc.

The dispersant nonpolar liquids (A) are, preferably, branched-chain aliphatic hydrocarbons and more particularly, Isopar ®-G, Isopar ®-H, Isopar ®-K, Isopar ®-L, and Isopar ®-M. These hydrocarbon liquids are narrow cuts of isoparaffinic hydrocarbon fractions with extremely high levels of purity. For example, the boiling range of Isopar ®-G is between 157° C. and 176° C., Isopar ®-H between 176° C. and 191° C., Isopar ®-K between 177° C. and 197° C., Isopar ®-L between 188° C. and 206° C. and Isopar ®-M between 207° C. and 254° C. Isopar ®-L has a mid-boiling point of approximately 194° C. Isopar ®-M has a flash point of 80° C. and an auto-ignition temperature of 338° C. Stringent manufacturing specifications, such as sulphur, acids, carboxyl, and chlorides are limited to a few parts per million. They are substantially odorless, possessing only a very mild paraffinic odor. They have excellent odor stability and are all manufactured by the Exxon Corporation. High-purity normal paraffinic liquids, Norpar ®12, Norpar ®13 and Norpar ®15, Exxon Corporation, may be used. These hydrocarbon liquids have the following flash points and auto-ignition temperatures:

| Liquid      | Flash Point (°C.) | Auto-Ignition Temp (°C.) |
|-------------|-------------------|--------------------------|
| Norpar ® 12 | 69                | 204                      |
| Norpar ® 13 | 93                | 210                      |
| Norpar ® 15 | 118               | 210                      |

All of the dispersant nonpolar liquids have an electrical volume resistivity in excess of  $10^9$  ohm centimeters and a dielectric constant below 3.0. The vapor pressures at 25° C. are less than 10 Torr. Isopar ®-G has a flash point, determined by the tag closed cup method, of 40° C., Isopar ®-H has a flash point of 53° C. determined by ASTM D 56. Isopar ®-L and Isopar ®-M have flash points of 61° C. and 80° C., respectively, determined by the same method. While these are the preferred dispersant nonpolar liquids, the essential characteristics of all suitable dispersant nonpolar liquids are the electrical volume resistivity and the dielectric constant. In addition, a feature of the dispersant nonpolar liquids is a low

Kauri-butanol value less than 30, preferably in the vicinity of 27 or 28, determined by ASTM D 1133. The ratio of thermoplastic resin to dispersant nonpolar liquid is such that the combination of ingredients becomes fluid at the working temperature.

Useful thermoplastic resins or polymers include: ethylene vinyl acetate (EVA) copolymers (Elvax® resins, E. I. du Pont de Nemours and Company, Wilmington, DE), copolymers of ethylene and an  $\alpha,\beta$ -ethylenically unsaturated acid selected from the class consisting of acrylic acid and methacrylic acid, copolymers of ethylene (80 to 99.9%)/acrylic or methacrylic acid (20 to 0%)/alkyl (C<sub>1</sub> to C<sub>5</sub>) ester of methacrylic or acrylic acid (0 to 20%), polyethylene, isotactic polypropylene (crystalline), ethylene ethyl acrylate series sold under the trademark Bakelite® DPD 6169, DPDA 6182 Natural and DTDA 9169 Natural by Union Carbide Corp., Stamford, CN; ethylene vinyl acetate resins, e.g., DQDA 6479 Natural and DQDA 6832 Natural 7 also sold by Union Carbide Corp.; Surlyn® ionomer resin by E. I. du Pont de Nemours and Company, Wilmington, DE, etc. Preferred copolymers are the copolymer of ethylene and an  $\alpha,\beta$ -ethylenically unsaturated acid of either acrylic acid or methacrylic acid. The synthesis of copolymers of this type are described in Rees U.S. Pat. No. 3,264,272, the disclosure of which is incorporated herein by reference. For the purposes of preparing the preferred copolymers, the reaction of the acid containing copolymer with the ionizable metal compound, as described in the Rees patent, is omitted. The ethylene constituent is present in about 80 to 99.9% by weight of the copolymer and the acid component in about 20 to 0.1% by weight of the copolymer. The acid numbers of the copolymers range from 1 to 120, preferably 54 to 90. Acid No. is milligrams potassium hydroxide required to neutralize 1 gram of polymer. The melt index (g/10 min) of 10 to 500 is determined by ASTM D 1238 Procedure A. Particularly preferred copolymers of this type have an acid number of 66 and 60 and a melt index of 100 and 500 determined at 190° C., respectively.

In addition, the resins have the following preferred characteristics:

1. Be able to disperse the colorant, e.g., pigment,
  2. Be insoluble in the dispersant liquid at temperatures below 40° C., so that the resin will not dissolve or solvate in storage,
  3. Be able to solvate at temperatures above 50° C.,
  4. Be able to be ground to form particles between 0.1  $\mu\text{m}$  and 5  $\mu\text{m}$ , in diameter,
  5. Be able to form a particle (average by area) of less than 10  $\mu\text{m}$ , e.g., determined by Horiba CAPA-500 centrifugal automatic particle analyzer, manufactured by Horiba Instruments, Inc., Irvine, CA: solvent viscosity of 1.24 cps, solvent density of 0.76 g/cc, sample density of 1.32 using a centrifugal rotation of 1,000 rpm, a particle size range of 0.01 to less than 10  $\mu\text{m}$ , and a particle size cut of 1.0  $\mu\text{m}$ .
  6. Be able to fuse at temperatures in excess of 70° C.
- By solvation in 3. above, the resins forming the toner particles will become swollen or gelatinous.

Suitable nonpolar liquid soluble ionic or zwitterionic compounds (C) include those compounds known in the art as agents that control the polarity of the charge on toner particles (charge directors). Examples of such compounds, which are generally used in an amount of 1 to 100 mg/g toner solids, are positive charge directors, e.g., sodium dioctylsulfosuccinate (manufactured by American Cyanamid Co.), zirconium octoate and metal

soaps such as copper oleate, etc.; negative charge directors, e.g., lecithin, barium petronate, calcium petronate (Witco Chemical Corp., New York, NY), alkyl succinimide (manufactured by Chevron Chemical Company of California), etc.

The fourth component of the electrostatic liquid developer is a polyhydroxy compound (D) which is preferably soluble in the developer in an amount of at least 2% by weight. Examples of this type compound which contain at least two hydroxyl groups include: ethylene glycol, 2,4,7,9-tetramethyl-5-decyn-4,7-diol, poly(propylene glycol), pentaethylene glycol, tripropylene glycol, triethylene glycol, glycerol, pentaerythritol, glycerol-tri-12 hydroxystearate, propylene glycerol monohydroxystearate, ethylene glycol monohydroxystearate, etc. The bulk conductivity which has proven particularly useful is in the range of about 1 to 80 pmho/cm.

The components are present in the electrostatic liquid developer in the indicated amounts.

- 20 Component A: 79 to 99.7% by weight, preferably 97.2 to 99.6% by weight;
- 21 Component B: 0.28 to 15.0% by weight, preferably 0.25 to 2.5% by weight;
- 22 Component C: 0.01 to 1.0% by weight, preferably 0.1 to 0.15% by weight; and
- 23 Component D: 0.01 to 5.0% by weight, preferably 0.05 to 0.15% by weight, all weights are based on the total weight of the developer.

As indicated above, additional components that can be present in the electrostatic liquid developer are colorants, such as pigments or dyes and combinations thereof, are preferably present to render the latent image visible, though this need not be done in some applications. The colorant, e.g., a pigment, may be present in the amount of up to about 60 percent by weight or more based on the weight of the resin. The amount of colorant may vary depending on the use of the developer. Examples of pigments are Monastral® Blue G (C.I. Pigment Blue 15 C.I. No. 74160), Toluidine Red Y (C.I. Pigment Red 3), Quindo® Magenta (Pigment Red 122), Indo® Brilliant Scarlet (Pigment Red 123, C.I. No. 71145), Toluidine Red B (C.I. Pigment Red 3), Watchung® Red B (C.I. Pigment Red 48), Permanent Rubine F6B13-1731 (Pigment Red 184), Hansa® Yellow (Pigment Yellow 98), Dalamar® Yellow (Pigment Yellow 74, C.I. No. 11741), Toluidine Yellow G (C.I. Pigment Yellow 1), Monastral® Blue B (C.I. Pigment Blue 15), Monastral® Green B (C.I. Pigment Green 7), Pigment Scarlet (C.I. Pigment Red 60), Auric Brown (C.I. Pigment Brown 6), Monastral® Green G (Pigment Green 7), Carbon Black, Cabot Mogul L (black pigment C.I. No. 77266) and Stirling NS N 774 (Pigment Black 7, C.I. No. 77266).

Fine particle size oxides, e.g., silica, alumina, titania, etc.; preferably in the order of 0.5  $\mu\text{m}$  or less can be dispersed into the liquefied resin. These oxides can be used alone or in combination with the colorants. Metal particles can also be added.

The percent pigment in the thermoplastic resin is 1% to 50% by weight preferably 1 to 15% by weight.

The particles in the electrostatic liquid developer have an average by area particle size of less than 10  $\mu\text{m}$ , preferably the average by area particle size is less than 5  $\mu\text{m}$ . The resin particles of the developer may or may not be formed having a plurality of fibers integrally extending therefrom although the formation of fibers extending from the toner particles is preferred. The term "fibers" as used herein means pigmented toner

particles formed with fibers, tendrils, tentacles, threadlets, fibrils, ligaments, hairs, bristles, or the like.

The electrostatic liquid developer can be prepared by a variety of processes. For example, into a suitable mixing or blending vessel, e.g., attritor, heated ball mill, heated vibratory mill such as a Sweco Mill manufactured by Sweco Co., Los Angeles, CA, equipped with particulate media for dispersing and grinding, Ross double planetary mixer manufactured by Charles Ross and Son, Hauppauge, NY, etc., are placed the above-described ingredients. Generally the resin, dispersant nonpolar liquid and optional colorant are placed in the vessel prior to starting the dispersing step although after homogenizing the resin and the dispersant nonpolar liquid the colorant can be added. Polar additive can also be present in the vessel, e.g., 1 to 99% based on the weight of polar additive and dispersant nonpolar liquid. The dispersing step is generally accomplished at elevated temperature, i.e., the temperature of ingredients in the vessel being sufficient to plasticize and liquefy the resin but being below that at which the dispersant nonpolar liquid or polar additive, if present, degrades and the resin and/or colorant decomposes. A preferred temperature range is 80° to 120° C. Other temperatures outside this range may be suitable, however, depending on the particular ingredients used. The presence of the irregularly moving particulate media in the vessel is preferred to prepare the dispersion of toner particles. Other stirring means can be used as well, however, to prepare dispersed toner particles of proper size, configuration and morphology. Useful particulate media are particulate materials, e.g., spherical, cylindrical, etc. taken from the class consisting of stainless steel, alumina, ceramic, zirconium, silica, and sillimanite. Carbon steel particulate media is useful when colorants other than black are used. A typical diameter range for the particulate media is in the range of 0.04 to 0.5 inch (1.0 to ~13 mm).

Suitable polar liquids which have a Kauri-butanol value of at least 30 include: aromatic hydrocarbons of at least 6 carbon atoms, e.g., benzene, toluene, naphthalene, other substituted benzene and naphthalene compounds; monohydric, dihydric and trihydric alcohols of 1 to 12 carbon atoms and more, e.g., methanol, ethanol, butanol, propanol, dodecanol, etc., ethylene and other glycols, Cellosolve; etc.

After dispersing the ingredients in the vessel, with or without a polar additive present until the desired dispersion is achieved, typically 1 hour with the mixture being fluid, the dispersion is cooled, e.g., in the range of 0° C. to 50° C. Cooling may be accomplished, for example, in the same vessel, such as the attritor, while simultaneously grinding in the presence of additional liquid with particulate media to prevent the formation of a gel or solid mass; without stirring to form a gel or solid mass, followed by shredding the gel or solid mass and grinding, e.g., by means of particulate media in the presence of additional liquid; or with stirring to form a viscous mixture and grinding by means of particulate media in the presence of additional liquid. Additional liquid means dispersant nonpolar liquid, polar liquid or combinations thereof. Cooling is accomplished by means known to those skilled in the art and is not limited to cooling by circulating cold water or a cooling material through an external cooling jacket adjacent the dispersing apparatus or permitting the dispersion to cool to ambient temperature. The resin precipitates out of the dispersant during the cooling. Toner particles of

average particle size (by area) of less than 10  $\mu\text{m}$ , as determined by a Horiba CAPA-500 centrifugal particle analyzer described above or other comparable apparatus, are formed by grinding for a relatively short period of time. In a grinding time of about 2 hours or less using polar liquid, particles in the average size (by area) of 0.1 to 5  $\mu\text{m}$  are achieved.

After cooling and separating the dispersion of toner particles from the particulate media, if present, by means known to those skilled in the art, it is possible to reduce the concentration of the toner particles in the dispersion, impart an electrostatic charge of predetermined polarity to the toner particles, or a combination of these variations. The concentration of the toner particles in the dispersion is reduced by the addition of additional dispersant nonpolar liquid as described previously above. The dilution is conducted to reduce the concentration of toner particles to between 0.1 to 3 percent by weight, preferably 0.5 to 2 weight percent with respect to the dispersant nonpolar liquid. One or more nonpolar liquid soluble ionic or zwitterionic compounds, of the type set out above, can be added to impart a positive or negative charge, as desired. The addition may occur at any time during the process. If a diluting dispersant nonpolar liquid is also added, the ionic or zwitterionic compound can be added prior to, concurrently with, or subsequent thereto. If the polyhydroxy compound has not been previously added in the preparation of the developer, it can be added subsequent to the developer being charged, as illustrated in Example 5 below. Preferably the polyhydroxy compound is present during the dispersing step. A preferred mode of the invention is described in Example 1.

#### INDUSTRIAL APPLICABILITY

The electrostatic liquid developers of this invention demonstrate improved charging qualities over liquid toners containing standard charge directors or other known additives. The toners of this invention are useful in copying, e.g., making office copies of black and white as well as various colors; or color proofing, e.g., a reproduction of an image using the standard colors: yellow, cyan, magenta together with black as desired. In copying and proofing the toner particles are applied to a latent electrostatic image.

Other uses are envisioned for the electrostatic liquid developers include: digital color proofing, which requires toners having high particle mediated conductivity, lithographic printing plates, and resists.

#### EXAMPLES

The following controls and examples wherein the parts and percentages are by weight illustrate but do not limit the invention. In the examples the melt indices were determined by ASTM D 1238, Procedure A, and the average particle sizes by area were determined by a Horiba CAPA-500 centrifugal particle analyzer as described above.

#### CONTROL 1

In a Union Process 01 Attritor, Union Process Company, Akron, Ohio, was placed the following ingredients:

| Ingredient                                              | Amount (g) |
|---------------------------------------------------------|------------|
| Copolymer of ethylene (89%) and methacrylic acid (11%), | 30.0       |

-continued

| Ingredient                           | Amount (g) |
|--------------------------------------|------------|
| melt index at 190° C. is 100,        |            |
| Acid No. is 66                       |            |
| Mogul ® L carbon black               | 8.0        |
| C.I. Pigment 77266, Cabot Corp.,     |            |
| Carbon Black Division, Boston, Mass. |            |
| Isopar ®-L, nonpolar liquid having a | 125.0      |
| Kauri-butanol value of 27, Exxon     |            |
| Corporation                          |            |

The ingredients were heated to 90° C.±10° C. and milled at a rotor speed of 230 rpm with 0.1875 inch (4.76 mm) diameter stainless steel balls for one hour. The attritor was cooled to room temperature while the milling was continued and then 125 grams of Isopar ®-H, nonpolar liquid having a Kauri-butanol value of 27, Exxon Corporation were added. Milling was continued and the average particle size by area was monitored. The particulate media were removed and the dispersion of toner particles was then diluted to 2 percent solids with additional Isopar ®-H and a charge director, 1.2 g of Basic Barium Petronate ® Sonneborn Division of Witco Chemical Corp., New York, N.Y. were added. Image quality was determined using a Savin 870 copier at standard mode: Charging corona set at 6.8 kV and transfer corona set at 8.0 kV using carrier sheets such as Savin 2200 paper, Plainwell off-set enamel paper number 3 gloss 60 lb. test, Plainwell Paper Co., Plainwell, MI. Conductivity results are shown in Table 2 below.

#### CONTROL 2

Example 1 was repeated with the following exceptions: 2.6 grams of Monastral ® Blue BT 383D were added in place of the Mogul ® L carbon black. Extremely poor image quality was obtained in a Savin 870 copier after charging with 1.8 g of barium petronate described in Control 1 or 1.2 g of lecithin. Results are shown in Table 2 below.

#### EXAMPLE 1

The procedure of Control 1 was repeated with the following exceptions: 2.6 grams of Monastral ® Blue BT 383D, C.I. Pigment No. 74160, manufactured by Du Pont, were used instead of carbon black and 6 grams of ethylene glycol were added before milling. After charging with 1.96 g of barium petronate described in Control 1 or 1.6 g lecithin, very good image quality was obtained using a Savin 870 copier at standard mode described in Control 1. Results are shown in Table 2 below.

#### EXAMPLE 2

In a Union Process 1-S Attritor, Union Process Company, Akron, Ohio was placed the following ingredients:

| Ingredient                                                                            | Amount (g) |
|---------------------------------------------------------------------------------------|------------|
| Copolymer of ethylene (89%) and methacrylic acid (11%), melt index at 190° C. is 100, | 200.0      |
| Acid No. is 66                                                                        |            |
| Monastral ® Blue BT 383D, Pigment Blue 15, C.I. No. 74160                             | 15.1       |
| Isopar ®-L, nonpolar liquid having a Kauri-butanol value of 27, Exxon Corporation     | 1000.0     |

-continued

| Ingredient      | Amount (g) |
|-----------------|------------|
| Ethylene glycol | 15.0       |

The ingredients were heated to 90° C.±10° C. and milled at a rotor speed of 230 rpm with 0.1875 inch (4.76 mm) diameter stainless steel balls particulate media for one hour. The attritor was cooled to room temperature while the milling was continued and then 700 grams of Isopar ®-H, nonpolar liquid having a Kauri-butanol value of 27, Exxon Corporation were added. Milling was continued and the average particle size by area was monitored. The particulate media were removed and the dispersion of toner particles was then diluted to 2 percent solids by weight with additional Isopar ®-H and a charge director such as 1.25 g of lecithin were added. Very good image quality was obtained using a Savin 870 copier at standard mode described in Control 1. Results are shown in Table 2 below.

#### EXAMPLE 3

The procedure of Control 2 was repeated with the following exception: 6 grams of Surfynol ®104E manufactured by Air Products and Chemicals, Inc., 50% 2,4,7,9-tetramethyl-5-decyn-4,7-diol in ethylene glycol were added before milling. After charging with barium petronate described in Control 1, very good image quality was obtained using a Savin 870 copier at standard mode described in Control 1. Conductivity results are shown in Table 2 below.

#### EXAMPLE 4

The procedure of Control 2 was repeated with the following exception: 6 grams of 2,4,7,9-tetramethyl-5-decyn-4,7-diol were added before milling. After charging with 1.9 g of barium petronate described in Control 1, image quality obtained using a Savin 870 copier at standard mode described in Control 1 was found to be better than that obtained with Control 2 toners. Results are shown in Table 2 below.

#### EXAMPLE 5

Four toners were prepared as described in Control 2, 25 mL of each diluted (2% solids) toner were then charged with 200 milligrams of 5.5 percent barium petronate. To three of the charged toners, 0.25 gram of the diols listed in Table 1 were added. Particle mediated conductivity was then measured. The toner sample containing no diol had no particle mediated conductivity. Particle mediated conductivities for the other three toners are shown in Table 1.

TABLE 1

| DIOL                   | PARTICLE<br>MEDIATED<br>CONDUCTIVITY<br>pmo/cm |
|------------------------|------------------------------------------------|
| Poly(propylene glycol) | 25                                             |
| Pentaethylene glycol   | 3                                              |
| Tripropylene glycol    | 3                                              |

#### COMPARATIVE EXAMPLE 1

The procedure described in Control 2 was repeated with the following exception: 6 grams of 7-ethyl-2-methyl-4-undecanol, which is the alcohol preferred in U.S. Pat. No. 4,457,995 and is a single alcohol with

more than 10 carbon atoms, were added before milling. When charged as described in Examples 1 and 3 no particle mediated conductivity was observed, and the toner could not be charged to give positive images using a Savin 870 copier at standard mode described in Control 1. Conductivity results are shown in Table 2 below.

#### COMPARATIVE EXAMPLE 2

Example 1 was repeated with the following exceptions: 2.25 grams of Dalamar® Yellow (Pigment Yellow 74, C.I. No. 11741) were added in place of the Monastral® Blue BT 383D. No charge director was added. Image quality was found to be very poor. Conductivity results are shown in Table 2 below.

#### COMPARATIVE EXAMPLE 3

Comparative Example 2 was repeated with the following exception: 54 grams of abietic acid were added before milling as described in Example III of U.S. Pat. No. 3,578,593. A very poor image was obtained. Conductivity results are shown in Table 2 below.

TABLE 2

| EXAMPLE           | CHARGE<br>DIRECTOR | CONDUCTIVITY <sup>1</sup> |      |      |
|-------------------|--------------------|---------------------------|------|------|
|                   |                    | BULK                      | SOLN | PART |
| Control 1         | Barium             | 60                        | 50   | 10   |
|                   | Petronate          | 74                        | 60   | 14   |
| Control 2         | Barium             | 11                        | 11   | 0    |
|                   | Petronate          |                           |      |      |
| 1                 | Lecithin           | 32                        | 32   | 0    |
|                   | Barium             | 49                        | 20   | 29   |
| 2                 | Petronate          |                           |      |      |
|                   | Lecithin           | 60                        | 40   | 20   |
| 3                 | Lecithin           | 69                        | 48   | 21   |
|                   | Barium             | 56                        | 45   | 11   |
| 4                 | Petronate          |                           |      |      |
|                   | Barium             | 19                        | 14   | 5    |
| Comparative Ex. 1 | Petronate          |                           |      |      |
|                   | Barium             | 13                        | 13   | 0    |
| Comparative Ex. 2 | Petronate          |                           |      |      |
|                   | Barium             | 0                         | 0    | 0    |
| Comparative Ex. 3 | Petronate          |                           |      |      |
|                   | Barium             | 0                         | 0    | 0    |
|                   | Petronate          |                           |      |      |

<sup>1</sup>Conductivities are measured in picomhos (pmho)/cm at five hertz and low voltage, 5.0 volts.

I claim:

1. An electrostatic liquid developer having improved charging characteristics consisting essentially of  
(A) nonpolar liquid having a Kauri-butanol value of less than 30, present in a major amount,

- 9
- 10
- (B) thermoplastic resin particles having an average by area particle size of less than 10  $\mu\text{m}$ ,  
(C) nonpolar liquid soluble ionic or zwitterionic compound, and  
(D) a polyhydroxy compound.
- 5 2. An electrostatic liquid developer according to claim 1 wherein the polyhydroxy compound is soluble in the developer in an amount of at least 2% by weight.
- 10 3. An electrostatic liquid developer according to claim 1 wherein component (A) is present in 79 to 99.7% by weight, component (B) is present in 0.28 to 15.0% by weight, component (C) is present in 0.01 to 1.0% by weight, and component (D) is present 0.01 to 5.0% by weight, all weight percentages being based on the total weight of the developer.
- 15 4. An electrostatic liquid developer according to claim 1 containing up to about 60% by weight of a colorant.
- 20 5. An electrostatic liquid developer according to claim 4 wherein the colorant is a pigment.
6. An electrostatic liquid developer according to claim 4 wherein the percent pigment in the thermoplastic resin is 1% to 50% by weight.
- 25 7. An electrostatic liquid developer according to claim 4 wherein the colorant is a dye.
8. An electrostatic liquid developer according to claim 1 wherein a fine particle size oxide is present.
- 30 9. An electrostatic liquid developer according to claim 1 wherein the thermoplastic resin is a copolymer of ethylene and an  $\alpha,\beta$ -ethylenically unsaturated acid selected from the group consisting of acrylic acid and methacrylic acid.
- 35 10. An electrostatic liquid developer according to claim 1 wherein the thermoplastic resin is an ethylene vinyl acetate copolymer.
11. An electrostatic liquid developer according to claim 1 wherein the thermoplastic resin is a copolymer of ethylene (80 to 99.9%)/acrylic or methacrylic acid (20 to 0%)/alkyl ester of acrylic or methacrylic acid wherein alkyl is 1 to 5 carbon atoms (0 to 20%).
- 40 12. An electrostatic liquid developer according to claim 9 wherein the thermoplastic resin is a copolymer of ethylene (89%)/methacrylic acid (11%) having a melt index at 190° C. of 100.
- 45 13. An electrostatic liquid developer according to claim 1 wherein the particles have an average by area particle size of less than 5  $\mu\text{m}$ .
14. An electrostatic liquid developer according to claim 1 wherein component (C) is barium petronate.
- 50 15. An electrostatic liquid developer according to claim 1 wherein component (C) is lecithin.

\* \* \* \* \*